

# UNITED STATES PATENT OFFICE.

RALPH DEANE ASLATT, OF MARTINEZ, CALIFORNIA.

## COMPOSITION FOR COATING BOILERS AND PIPES.

1,372,664.

Specification of Letters Patent. Patented Mar. 29, 1921.

No Drawing.

Application filed May 20, 1920. Serial No. 382,904.

To all whom it may concern:

Be it known that I, RALPH DEANE ASLATT, a subject of the King of Great Britain, residing at Martinez, in the county of Contra Costa and State of California, have invented 5 certain new and useful Improvements in Compositions for Coating Boilers and Pipes; and I do declare the following to be a full, clear, and exact description of the invention, 10 such as will enable others skilled in the art to which it appertains to make and use the same.

This invention relates to plastic coating compositions, and more specifically to an 15 improved composition for coating boilers and pipes for heat insulating purposes.

Several objects of this invention are to provide a coating composition of this character which can be manufactured at an exceedingly 20 low cost, can be kept a very great length of time without spoiling, and is very quickly and easily prepared, by mixing with cold water, so that the maximum convenience is obtained at the minimum cost.

25 A further object is to provide a dry or comparatively dry composition which, when properly mixed with water, is very easily applied, being very adhesive, and which, when applied, will not corrode or cause corrosion 30 to the surface coated therewith, is quite hard when set and dry, does not crack from shrinking, is fire-proof, and is sufficiently porous to permit steam or water to pass therethrough, so that any leak in the 35 surface coated therewith can be easily detected and located.

Other objects and advantages will be pointed out or implied in the following details of description:

40 In preparing this composition, the best results appear to be obtained by mixing,— 2 parts, by measure, of powdered or comminuted dry chalk; 1 part, by measure, of powdered or com- 45 minuted dry clay; 9 parts, by measure, of comminuted or loose vegetable pulp-fiber; 9 parts, by measure, of comminuted or loose textile fiber. 50 In practice, the clay may be of the kind obtained either from dry land or from the beds of rivers and other bodies of water, the essential feature being that it produces 55 a plastic or adhesive material when mixed with the proper quantity of water or other liquid. The vegetable pulp fiber may be

of the kind obtained from wood, or other vegetation and, for the sake of comparative cheapness, it is found advantageous to utilize waste paper, pasteboard, etc. The textile fiber may consist of wool, hair, cotton or other vegetable fiber having length and strength sufficient to be woven or fabricated; but, for the sake of comparative cheapness, this textile fiber is preferably obtained from 60 old rags, old rope, etc.

Where the composition is to be used immediately, or to be shipped in air-tight containers for subsequent use, the comminuted chalk and fiber may be mixed with the mud 70 or clay in the plastic state of the latter, so that little or no water need be added to give the composition the proper plastic consistency. However, for the sake of comparative cheapness, where the composition is to 75 be handled as an article of merchandise in large quantities, it is preferable to mix the ingredients dry, after being reduced to powder or granules and lint, whereupon, this dry mixture may be placed in bags, barrels, 80 hogsheads or boxes, or may be shipped loose in cars or other conveyances to dealers and consumers.

The term "comminuted," as applied to vegetable pulp fiber and textile fiber, is intended to distinguish from such fibers in a woven or fabricated state, or in other words, it is intended to distinguish between fiber in an interengaged state and fiber in the state where the fiber-strands are separated or 90 disengaged from one another.

Where the composition is in the dry state, it must be prepared for use by mixing it with a sufficient quantity of water or other liquid to produce a plastic material of the 95 consistency of common mortar, and it may be applied in successive coats, one upon the other, by means of the hand or by any appropriate means. Where a comparatively small surface is to be coated, such as a steam- 100 pipe or a small boiler, the user may apply the first one or two coats with his hands, dabbing the first coat on roughly so as to obtain a secure foundation for the subsequent coats. When the first coat has dried, 105 the second coat can be laid, pressed and evened with the hand, and when a third coat is desirable, this may either be applied with the hand or a trowel, and should be smoothed with a trowel where a smooth surface is 110 desirable. If it is desirable that the surface be very smooth and even, it should be trow-

eled after it has dried considerably, but before it has entirely dried. A thickness of two inches may be obtained with 3 coats, as no appreciable shrinking or cracking of the aggregate coat need be apprehended. When applying the first coat, the surface of the pipe or boiler should not be too hot, and to avoid overheating of the pipe, the steam pressure should not exceed 10 pounds. However, when the third coat is applied, the pressure should be as great as the normal working pressure.

It is not intended to limit this invention to the exact ingredients and proportions specified in the foregoing, but changes may be made within the scope of the inventive idea as implied and claimed.

What I claim as my invention is:

1. The composition to be mixed with liquid for producing a plastic coating mate-

rial, comprising a dry mixture of comminuted clay, comminuted chalk, and comminuted fiber.

2. The composition for mixing with liquid to produce a plastic coating material, comprising the following ingredients by measure, viz., 2 parts comminuted chalk, 1 part comminuted dry clay, 9 parts comminuted vegetable pulp-fiber, 9 parts comminuted textile fiber.

3. A plastic coating composition comprising by measure, two parts comminuted chalk, one part comminuted clay, nine parts comminuted vegetable pulp-fiber, and nine parts comminuted textile fiber.

In testimony whereof I have hereunto set my hand.

RALPH DEANE ASLATT.

Witness:

B. L. BOYER.